

# UNITED STATES PATENT OFFICE.

JAQUES EDWIN BRANDENBERGER, OF PARIS, FRANCE, ASSIGNOR TO LA SOCIETE LA CELLOPHANE, OF PARIS, FRANCE.

## SENSITIVE CELLULOSIC FILM AND PROCESS FOR PRODUCING THE SAME.

1,404,737.

Specification of Letters Patent.

Patented Jan. 31, 1922.

No Drawing.

Application filed March 7, 1921. Serial No. 450,400.

To all whom it may concern:

Be it known that I, JAQUES EDWIN BRANDENBERGER, citizen of the Republic of Switzerland, and resident of Paris, France, 5 post-office address 16 Rue du Louvre, have invented a new and useful Sensitive Cellulosic Film and Process for Producing the Same, which improvements are fully set forth in the following specification.

10 This invention relates to photographic films which are permeable to water and to a process for the preparation of the same.

Up to the present when photographic films which are permeable to water such as 15 cellulose (viscose) films were being prepared a sensitive salt, for example silver bromide had to be formed by successively treating the film in two baths, for example one containing silver nitrate and the other 20 potassium bromide, the silver bromide sensitive to light being formed in the interior of the mass. The silver bromide could not be made to penetrate the interior of the film by means of a silver bromide bath, because 25 this substance is not soluble in water and it is well known that water is necessary in the preparation of photographic films from materials which are permeable to water.

The operation may be simplified by using 30 a single bath in the following manner:

Silver iodide for example,—which is a sensitive salt of the same category as the bromide—is insoluble in water but soluble in an aqueous solution of potassium iodide.

35 According to the present invention an aqueous solution of potassium iodide is prepared in which silver iodide is dissolved until the solution is saturated.

Thereupon the film is immersed in the 40 bath. As soon as it is sufficiently impregnated it is withdrawn and squeezed and then soaked in water. The resulting dilution of the potassium iodide solution sets free a large quantity of silver iodide which 45 is deposited in the interior of the film and renders the latter sensitive.

The same result can be obtained by using

for example a warm solution of silver bromide in an alkaline bromide.

What I claim and desire to secure by Letters Patent is:—

1. The process for the production of sensitive cellulosic films for photographic purposes, which consists in impregnating the film with a solution of a silver halogen salt 55 in a suitable solvent, and thereupon precipitating the said silver halogen salt within the said film by the action of a suitable liquid.

2. The process for the production of sensitive cellulosic films for photographic purposes, which consists in impregnating the film with a solution of a silver halogen salt in a suitable solvent, and thereupon precipitating the said silver halogen salt within 65 the said film by the action of water.

3. The process for the production of sensitive cellulosic films for photographic purposes, which consists in impregnating the film with a solution of a silver halogen salt 70 in an alkali-halogen salt by heating if desired, squeezing the impregnated film and thereupon precipitating the said silver halogen salt within the said film by the action of water.

4. The process for the production of sensitive cellulosic films for photographic purposes, which consists in impregnating the film with a solution of silver iodide in potassium iodide, squeezing the impregnated 80 film and thereupon precipitating the said silver iodide within the said film by the action of water.

5. A sensitive cellulosic film for photographic purposes, essentially characterized 85 by the fact that the entire film is impregnated with a sensitive salt of silver.

In testimony whereof I have signed this specification in the presence of two subscribing witnesses.

JAQUES EDWIN BRANDENBERGER.

Witnesses:

GEORGES PASCAL CARRIÈRE,  
GERMAINE MICHIEL'S.